

## UNITED STATES PATENT OFFICE

1,932,381

METHOD OF TREATING LUBRICATING OILS  
AND THE PRODUCTS RESULTING THEREFROMBenjamin Gallsworthy, Bayonne, N. J., assignor  
to The Texas Company, New York, N. Y., a corporation of DelawareNo Drawing. Application May 9, 1930  
Serial No. 451,205

2 Claims. (Cl. 87—9)

This invention relates to methods of treating compounded lubricating oils or the separate constituents prior to the compounding thereof, and it is an object of my invention to produce a compounded lubricating oil having a high lubricating value.

It has been determined that lubricating oils can be improved to a marked degree by compounding therewith a relatively small amount of oxidized paraffin wax. Experiments have indicated that varying amounts of the oxidized wax may be used but compounded oils containing about 2% of such wax have been found to give satisfactory results. Oils so compounded ordinarily have a comparatively high acid value. For example, where compounded oils have been made up of 250 pale oil with two per cent of oxidized paraffin wax taken from different batches, it has been found that the acid values of the compounded oils have varied from 1.08 to 1.70, depending upon the particular characteristics of the oxidized paraffin wax used.

Lubricating oils having acid values as high or possibly higher than those indicated above may be entirely satisfactory for certain purposes, but in many instances it is desirable to use oils having relatively low acid values and in such cases it is possible to treat oils having high acid values to reduce the acid values and thereby provide oils having the desired characteristics.

I have found that the acid value of a lubricating oil compounded with a relatively small amount of oxidized paraffin wax can be materially decreased by treating the compounded oil with an adsorbent material such as decolorizing clay of the type of fuller's earth while maintaining it at a temperature of from 120° to 140° F. Oil compounded with two per cent of oxidized paraffin wax has been treated in the manner just described with the result that the acid value has been reduced to between 0.30—0.48, which is a marked decrease from the 1.08—1.70 acid value before the treatment.

My invention also contemplates the treatment

of oxidized paraffin wax prior to compounding it with filtered lubricating oil stock. The oxidized wax may be cut back with a volatile diluent such as naphtha or light gasoline to render it suitable for treatment with the adsorbent material and the diluent can be subsequently removed, or the wax may be treated in a more concentrated form, if preferred, due to the fact that the clay treatment is effected with sufficient heat to reduce the wax to a liquid or semi-liquid condition. In carrying out the invention in this manner the wax is first treated with an adsorbent material to effect a decrease in its acid value and the treated wax is then compounded with the lubricating oil stock to produce an oil having a high lubricating value.

This invention is not limited to the treatment of oils compounded with any specific quantity of oxidized paraffin wax or at any specific degree of heat, for experiments have shown that from one to five per cent of wax can be used with entirely satisfactory results and that the temperature may be varied throughout a considerable range. Other modifications of the invention may suggest themselves to those skilled in the art, and I desire therefore to be limited only as indicated in the appended claims.

I claim:

1. A method of producing a lubricating oil having an acid value of less than .5%, which comprises treating oxidized paraffin wax with fuller's earth while maintaining it at a temperature sufficient to keep it in a liquid state to reduce its acid value and thereafter compounding the treated wax with lubricating oil stock in the proportion of 1 to 5%.

2. A method of producing a lubricating oil having an acid value of less than .5%, which comprises cutting back oxidized paraffin wax with a volatile diluent, treating the cut-back wax with fuller's earth, while maintaining it at a temperature of about 120 to 140° F., removing the diluent and finally compounding the treated wax with lubricating oil stock in the proportions of 1 to 5%.

BENJAMIN GALLSWORTHY.

45

100

50

105

55

110